

July 9, 1935.

R. HARDING, JR

2,007,945

ELECTRIC LAMP WITH CONCENTRATED LIGHT SOURCE

Filed Sept. 16, 1930



Fig. 2.



Fig. 3.



INVENTOR  
ROBERT HARDING JR.  
BY  
Chester A. Barcelon  
ATTORNEY

## UNITED STATES PATENT OFFICE

2,007,945

ELECTRIC LAMP WITH CONCENTRATED  
LIGHT SOURCE

Robert Harding, Jr., Elmsford, N. Y., assignor to  
Sirian Lamp Company, Newark, N. J., a corporation of Delaware

Application September 16, 1930, Serial No. 482,243

## 5 Claims. (Cl. 176—1)

This invention relates to electric lamps of the gaseous discharge type.

In the application of Chester H. Braselton, entitled "Electrical discharge device", Serial No. 5 459,048, filed June 3, 1930, an electric lamp is described in which an electron emitting element is heated by passing a current therethrough in the presence of an ionizable gas at a pressure sufficient to confine the ionization of the gas to the region of the electron emitting element. When the electron emitting element is energized a brilliant bluish-white discharge in the nature of a halo appears along the electron emitting element forming a conductive path out- 10 side of the element and producing a bright uniform light. In this device, however, a resistance wire is necessary and it is somewhat difficult to get a resistance wire which will be heated to the correct temperature and have the proper 15 resistance when used with 110 volts so that a relatively long filament may be necessary to take the voltage. This necessitates a spreading out of the light source over a relatively large area.

It is therefore one of the objects of the present 20 invention to provide an electric gaseous discharge lamp with a concentrated light source.

Another object of the invention is to provide 25 an electric lamp in which illumination is produced not only by a gaseous discharge but by radiation from a refractory member which is heated by the discharge.

Another object of the invention is to provide 30 an electric lamp in which a refractory member is used to guide an ionic discharge so as to greatly increase the length of the discharge for a given 35 space.

Other objects of the invention and objects relating particularly to the construction and assembling of the various parts will be apparent 40 as the description of the invention proceeds.

Several embodiments of the invention have been illustrated in the accompanying drawing in which:

Fig. 1 is a side elevational view of my im- 45 proved electric lamp;

Fig. 2 is an enlarged longitudinal sectional view of the elements shown in Fig. 1;

Fig. 3 is an enlarged longitudinal sectional view of the electron emitting element; and

Fig. 4 is a longitudinal sectional view of a modified form of electron emitting element.

The lamp shown in Fig. 1 comprises an envelope 10, which may be formed integral with the usual press 11 for supporting the elements of the lamp. A cylinder 12 of refractory material such

as Nernst or Welsbach material may be supported by any suitable means such as by two rods 13 and 14 which may extend into the ends of the cylinder as indicated in Fig. 2. The rods 13 and 14 may be welded respectively to support rods 15 and 16 which may extend downwardly to the press 11 in which they may be sealed. Leading-in wires 17 and 18 may be connected respectively to the support rods 15 and 16.

The cylinder 12 is preferably provided with a 10 helical groove 19 which extends around the circumference from end to end forming a helical wall 20 the sides of which are separated by the spacing of the groove. Around the groove 19 I wind an electron emitting element 21 which may 15 be made of a coil 22 of resistance wire closely wound in concentrated form and the outer surface of which is coated with an electron emitting material 23. The resistance wire may be any desired resistance wire such as tungsten, molyb- 20 denum, tantalum, or nichrome and the electron emitting material 23 may be any of the well-known materials used for that purpose such as the oxides of the alkaline earth metal group, all of which have an electron emissivity when heated 25 in excess of that of thorium oxide, or mixtures of such materials but preferably the material should include one which has the property of selective radiation such as calcium oxide. Where the ends of the element 21 extend beyond the 30 ends of the cylinder 12 they may be welded to the support rods 15 and 16 to electrically connect the support rods with the element 21.

The bulb is filled with an inert gas or mixtures of such gases preferably those having a mon- 35 atomic structure such as neon, argon, helium, krypton, xenon, and the like. Also vapors of metals such as mercury, caesium, or rubidium may be mixed in small quantities with the other gases to increase the conductivity and to produce 40 color effects.

The metal vapor may be introduced into the bulb by providing a salt such as a chloride, of the desired metal together with a small quantity of magnesium in a suitable container 15a which 45 may be mounted by means of the wire 15b upon the support rod 15. When this container is heated as by external bombardment after the bulb is sealed off the magnesium flashes and forms magnesium chloride liberating the other metal which 50 condenses on the inner walls of the bulb. It evaporates again as soon as the bulb is heated in use.

When the current is turned on current will flow through the leading-in wire 17, through the sup- 55

- port rod 15, the element 21, the support rod 16, and out through the leading-in wire 18. This energizes the element 21 and raises the temperature thereof so that it becomes a good electron emitter.
- 5 The bombardment of the gas by the electrons apparently causes ionization thereof which produces a conductive path in the region of the element so that current will flow from one end of the element to the other along this conductive path.
- 10 Inasmuch as the adjacent turns of the element are separated by the wall 20 of refractory material there can be no short circuit of the discharge from one turn to another except over the edge of the wall 20. When the ionic discharge appears 15 it bombards the wall 20 and raises the temperature thereof until the refractory material radiates light and increases the total light output of the lamp. As the surface only is bombarded and as it is the surface that emits light there is no 20 temperature drop through the refractory material and more energy is therefore translated into light.
- When the discharge appears and the cylinder 12 becomes heated it also acts as a conductor 25 of electricity and a current will then flow through the cylinder 12 between the rods 13 and 14. This helps increase the temperature of the rod 12 but the large percentage of the current will flow in the element 21 and around the groove 19 following the path of the low resistance ionized gas 30 in the vicinity of the element.
- Care should be taken in exhausting the lamp that substantially all occluded gases are removed and pure gases are used to fill the envelope.
- 35 With the elements mounted as in Fig. 1 upon the press 11 and the press sealed in the envelope 10, the latter may be connected with a vacuum pump and covered by the usual oven for raising the temperature thereof to about 350 to 400° C. or to 40 as high a temperature as the glass will stand without deforming. Sufficient current may be run through the filament at this time to raise the temperature thereof to approximately 600° C. and the heating and evacuating are continued until 45 there is no fluorescence when high tension current from an induction coil is directed against the walls of the bulb or in other words until there is no more gas inside of the bulb. This process may be continued until a high vacuum of about .5 micron is obtained. The current may then be increased through the filament and the temperature thereof slowly raised until it is a bright red at 50 a temperature of about 800° C. This drives out the binder in the electron emitting material and other occluded gases which might be present.
- 55 When no more gas is found in the bulb the oven may then be raised and the filament heated for a moment to about 1200° C. the pump being connected all this time to maintain a high vacuum.
- 60 The pump may then be shut off and the filament current turned off and a slight amount of inert gas preferably neon at about  $\frac{1}{2}$  mm. pressure admitted into the bulb and the filament current then turned on again. Spots of localized discharge having a reddish color will then appear.
- 65 These spots gradually spread until a diffused glow completely fills the bulb. This process appears to activate the electron emitting coating and is maintained until the discharge is uniform throughout the entire bulb which usually takes less than ten minutes when the activation is completed.
- 70 During this time the current on the filament should not be raised too high so the coating will not be destroyed or thrown off from the filament.
- 75

If white discharge spots appear on the filament or the support rods, it is an indication that there are more gases or vapors in the bulb and the bulb is again preferably exhausted and the whole process of activation repeated.

5 When the activation is completed the filament temperature may be raised to about 1400° C., then the vacuum pump again connected and the gas pumped out to remove the undesirable gases which may have been thrown off during the activation 10 process. The filament circuit may then be disconnected, the pump turned off, and about 50 mm of neon gas followed by about 150 mm of argon may be admitted into the bulb. The bulb may then be sealed off and is ready for use.

15 It will be noted that the light is produced from several sources: the light produced by the filament itself, the light produced by the discharge which surrounds the filament, and the light produced by the refractory cylinder 12, and it will 20 be noted that inasmuch as the electron emitting element is wound around the cylinder 12 the space taken up is relatively small compared to the space it would take if the filament were stretched out in a straight line. Thus the region of the 25 light source is reduced to a minimum.

It may be desirable instead of using a coil of resistance wire, as indicated in Fig. 3, to use a single wire which may be wound around a smaller groove 25 provided in a refractory cylinder 26. If 30 desired the wire 24 may be coated with electron emitting material before winding in the groove or it may be wound first and the outer surface coated as indicated in Fig. 4.

If desired the pressure in the bulb may be 35 made sufficient so that there will be no discharge over the top of the wall 20 but the discharge will then be confined to a spiral path around the groove 19. However, the invention is intended to contemplate the extension of the 40 discharge far enough outwardly to permit short circuiting across the wall 20.

Many modifications of the invention may be resorted to without departing from the spirit thereof, and I do not therefore, desire to limit 45 myself to what has been shown and described except as such limitations occur in the appended claims.

What I claim is:

1. An electric lamp comprising an envelope, an 50 electron emitting element within said envelope so bent that portions thereof are nearer together across a gaseous space than along the conducting path of said element, the density of electron emission when heated being in excess of 55 that from thorium oxide, an ionizable gas surrounding said element and having a breakdown potential per unit length of element less than the potential along said unit length of element necessary to raise said element to electron emitting temperature, and means between said portions to hinder a current flow between said portions through said gas.

2. An electric lamp comprising an envelope, an 60 electron emitting element within said envelope, the density of electron emission when heated being in excess of that from heated thorium oxide, an ionizable gas surrounding said element and having a breakdown potential per unit length of said element only when said element 70 is subjected to electron bombardment which is less than the potential across said unit length necessary to raise said element to electron emitting temperature whereby a layer of ionized gases is formed about the element when heated, and 75

means between portions of said element to limit flow of current from one portion to the other through contact from adjacent layers of ionized gas, said electron emitting element forming the sole source of the discharge.

3. An electric lamp comprising an envelope, an electron emitting element within said envelope, the density of electron emission when heated being in excess of that from heated thorium oxide, an ionizable gas surrounding said element and having a breakdown potential per unit length of said element only when said element is subjected to electron bombardment which is less than the potential along said unit length necessary to raise said element to electron emitting temperature whereby a layer of ionized gases is formed about the element when heated, and means to separate the ionized gas layer adjacent one portion of said element from the ionized layer of gas adjacent another portion of said element to prevent a current discharge between said two portions through said gas layer, said electron emitting element forming the sole source of the discharge.
- 10 4. An electric lamp comprising an envelope, an electron emitting element containing an oxide of the alkaline earth metal group within said envelope wound in the form of a coil, an ionizable

gas surrounding said element and having a pressure sufficient to confine the ionization of said gas to the region of said element when said element is energized, and means between the turns of said coil to hinder a direct current path from one turn to another on the exterior of said coil when said filament is energized, said electron emitting element forming the sole source of the discharge.

5. An electric lamp comprising an envelope, a cylinder of refractory material within said envelope having the quality of selective radiation, a helical groove around the circumference of the cylinder, a filamentary resistance wire wound in said groove, a coating of an oxide of one of the alkali earth metals on said wire, the diameter of said wire and the coating being less than the depth of said groove, and an ionizable gas containing a mixture of neon and argon surrounding said wire and element and having a pressure sufficient to confine the ionization of said gas to the region of said wire when said wire is energized, whereby a layer of luminous gas is formed about the external surface of said cylinder, said coated resistance wire forming the sole source of the discharge.

ROBERT HARDING, JR.